

# United States Patent Office

2,800,443

Patented July 23, 1957

1

2,800,443

## METHOD OF CHROMIUM PLATING

Jesse E. Stareck, Royal Oak, Edgar J. Seyb, Jr., Oak Park, and Frank Passal, Detroit, Mich., assignors, by mesne assignments, to Metal & Thermit Corporation, New York, N. Y., a corporation of New Jersey

No Drawing. Application July 26, 1955,  
Serial No. 524,578

11 Claims. (Cl. 204—51)

This invention relates to an improved method for chromium plating hard, high strength steels. Conventional chromium plating of such steels is accompanied by such a high loss of fatigue strength that failure of the steel usually occurs under repeated loading; moreover, the loss in fatigue strength increases with increasing strength of the steel. This unfavorable effect of conventional chromium plating has naturally limited the usefulness of these plated steels.

A principal object of the invention is to provide a method for chromium plating hard, high strength steel without substantial loss of fatigue strength. The method is particularly directed to the plating of steel articles for use at ordinary temperatures under conditions of repeated stress and strain that approach the fatigue limit of the steel. It has been found that a high fatigue strength may be obtained in the plated article if the chromium deposited on it contains a large number of fine cracks such that it exhibits a low residual stress. The resultant chromium plated steel enjoys the protection against corrosion and wear, and the hardness and low resistance to friction, that the chromium deposit affords, and by virtue of the present improvement is suitable for use under service conditions involving repeated loading. Thus the field of application of the plated steel is enlarged.

The invention comprises electrodepositing chromium on an article of steel having a fatigue strength of at least 50,000 p. s. i. (pounds per square inch), and particularly 60,000 or 70,000 to 110,000 p. s. i., although steels of higher strength may be also plated. A current of  $\frac{1}{4}$  to 5 a. s. i. (ampères per square inch), preferably  $\frac{1}{4}$  to 3 a. s. i., is passed to the article as cathode in an aqueous bath having a chromic acid,  $\text{CrO}_3$ , content of 100 to 400 g./l., preferably 150 to 300 g./l., and containing dissolved sulfate,  $\text{SO}_4^{2-}$ , as catalyst. The ratio of  $\text{CrO}_3$  to dissolved  $\text{SO}_4^{2-}$  is 40:1 to 100:1, and the bath temperature is 90 to 110° F. A wider temperature range, namely, 90 to 130° F., may be employed for baths having a  $\text{CrO}_3/\text{SO}_4^{2-}$  ratio of 40:1 to 85:1. Chromium is plated on the article to form a coating at least 1 mil thick.

The chromic acid may be supplied to the bath as such and the sulfate in the form of any suitable compound, such as sulfuric acid.

At  $\text{CrO}_3$  concentrations of 300 to 400 g./l. the bath may be made to be self-regulating with respect to the sulfate concentration. Such a bath comprises  $\text{CrO}_3$  and, as the source of the sulfate, calcium sulfate in an amount sufficient to saturate the bath and to provide an undissolved excess of calcium sulfate. As this saturation concentration of dissolved sulfate is higher than required, a soluble calcium compound is added in an amount sufficient to suppress the concentration of dissolved sulfate from its unsuppressed saturation concentration to a lower value corresponding to the required  $\text{CrO}_3/\text{SO}_4^{2-}$  ratio. Thus, as dissolved sulfate is removed from the bath, as by drag out losses, sufficient excess calcium sulfate goes into solution to replace the lost sulfate. Lower temperatures and ratios are preferred for this type of bath; thus, in the case of a  $\text{CrO}_3$  concentration of 300 g./l., a ratio of 40:1 to 60:1 is quite satisfactory. Suitable soluble

2

calcium suppressor compounds for providing dissolved calcium are calcium oxide, calcium hydroxide, calcium carbonate, calcium dichromate, and calcium chromate. For example, for baths containing 400 g./l. of  $\text{CrO}_3$  there is added sufficient calcium sulfate to the solution to saturate it and then 7 g./l. of dissolved suppressor calcium are added to give a ratio of  $\text{CrO}_3$  to  $\text{SO}_4^{2-}$  of 40 to 1; 14 g./l. of dissolved suppressor calcium are added to give a ratio of 60 to 1; 20 g./l. for a ratio of 80 to 1; and 25 g./l. for a ratio of 100 to 1. For baths containing 300 g./l. of  $\text{CrO}_3$  a 40 to 1 ratio and a 60 to 1 ratio can be obtained with 12 and 20 g./l., respectively, of dissolved suppressor calcium.

The unplated steel may have a Rockwell hardness of at least 20C. The upper limit of hardness may be as desired, for example up to 54C. Good results are obtainable with steels having a Rockwell hardness in the range of 28C to 47C, particularly 33C to 47C. Alloy or high quality steels are quite suitable for plating, but the invention is not limited to them. Substantial thicknesses of chromium are deposited on the steel, ranging from 1 or 2 to 30 or more mils, and preferably from 5 to 15 mils. Plating times may vary widely, for example from 1 to 24 or more hours.

Chromium electrodeposits exhibit the characteristic of stress, a property which changes with the thickness of the deposit and which, by means of a spiral contractometer, can be measured throughout the course of a plating operation. With this instrument the stress in a long continuous section of chromium plate is transferred to the underlying base metal comprising a long, helically wound strip of thin metal having one end free to rotate. The stress in the plate can be calculated from the amount of rotation. It has been found that initially, the stress in a deposit increases very rapidly during the first few moments of plating until it exceeds the tensile strength of the deposit, at which point crack-lines form in the chromium to relieve the high tensile stress. As the thickness of the plate increases, the stress gradually decreases, approaching zero stress, and the number of the crack-lines increases. The number of crack-lines may readily be determined by counting them as described below in Examples 1-8. The crack-lines become finer as their number increases. It has been further found in some cases that as the plate thickness increases, the stress decreases so that it becomes negative in value as distinguished from the positive values previously obtained. This behaviour is illustrated in Table 1 below which sets forth stress data, as obtained by the spiral contractometer, at various plate thicknesses for a bath whose composition and operating conditions are given in Example 7 of Table 3. It may be noted that in the plating run carried out at 2 a. s. i., the stress was already dropping by the time the first readings on the contractometer were taken.

Table 1

| Chromium thickness, mils | Stress, 1,000 p.s.i. |          |
|--------------------------|----------------------|----------|
|                          | 1 a.s.i.             | 2 a.s.i. |
| 0.025                    | 161                  | 175      |
| 0.05                     | 166                  | 159      |
| 0.1                      | 156                  | 157      |
| 0.2                      | 106                  | 130      |
| 0.3                      | 74                   | 87       |
| 0.4                      | 54                   | 64       |
| 0.5                      | 42                   | 47       |
| 0.75                     | 26                   | 31       |
| 1.0                      | 17                   | 20       |
| 1.5                      | 8                    | 10       |
| 2.0                      | 3                    | 5        |
| 2.5                      | 1                    | 2        |
| 3.0                      | 0                    | 0.5      |
| 3.5                      | —                    | —0.5     |
| 4.0                      | —                    | —1       |

A correlation exists between the stress and the number of crack-lines. As an illustration, three deposits were plated on steel specimens (described below in Examples 1-8) and exhibited the properties listed in Table 2. Each deposit was 2 mils thick. The three deposits were produced from baths described in Examples 7, 1, and 6.

Table 2

| Crack-lines per inch | Stress, 1,000<br>p.s.i. | 10 |
|----------------------|-------------------------|----|
| 1,200                | 3                       |    |
| 400                  | 40                      |    |
| 50                   | 47                      |    |

The more numerous the crack-lines, the lower is the measured stress, and conversely, the fewer the crack-lines, the higher the stress. The correlation applies over a wide stress range, varying from a positive tensile stress of about +80,000 p. s. i. to a negative compressive stress of -15,000 or -20,000 p. s. i. Between about -15,000 and -20,000 p. s. i. the stress tends to level off such that further increases in the number of crack-lines is not accompanied by more negative stress values. The correlation holds for thicker deposits, say those of at least 1 mil thickness. By counting the number of crack-lines in a deposit it is possible to obtain an indirect semi-quantitative measure of the stress in the deposit and to compare one deposit with another.

The number of crack-lines in chromium plate deposited on hardened high strength steel is also correlated with the fatigue strength of the plated steel, the more numerous the crack-lines, the higher being the fatigue strength. It follows that deposits exhibiting high tensile stress result in a severe lowering of the fatigue strength of the steel, whereas deposits of low stress give much less lowering of the fatigue strength. It is desirable to deposit on the steel a plate having 1000, preferably 1200, to 10,000 crack-lines per inch. In terms of stress, the plate should range from +5000 p. s. i. tensile stress, preferably 0 p. s. i., to -20,000 p. s. i. compressive stress. Steel plated with deposits of this character exhibit a higher fatigue strength than if plated with deposits not so characterized. Fatigue strengths of about 70%, and more, of the unplated steel are obtainable, with strengths of at least 85% being preferred. Strengths of 60 to 70% of the unplated steel are satisfactory for many purposes.

The crack pattern of a deposit is determined early in the plating operating, say after about 0.5 mil of chromium is deposited. A consequence of this fact is that an article may be plated to a point where a desirable crack pattern, i. e., numerous crack-lines, has been established and then transferred to another bath of the same type but operated at a higher speed, so that a desirable plate of required thickness may be obtained in a shorter time. Another characteristic of the method is that the crack pattern of a deposit may be favorably changed during plating as by periodically reversing the current.

An incident of the chromium plating of steel in chromic acid plating baths is the embrittlement of the steel by hydrogen released during the plating operation. Where embrittlement of the chromium plated steel is a factor to be considered in connection with the end use of the steel, it can be prevented or substantially minimized by applying a barrier metal such as a copper strike between the steel and the chromium. Copper strike films may be applied by plating the steel in a suitable copper plating bath for a short time to deposit about 0.01 to 0.1 or 0.2 mil of copper. The fatigue strength of the resulting copper plated, chromium plated steel, by comparison with a like steel similarly chromium plated but not copper plated, is not affected by the presence of the copper barrier. Suitable copper plating baths include conventional cyanide copper baths and copper sulfate-sulfuric acid baths, as described in "Principles of Electroplating and Electro-

forming," Blum and Hogboom, revised 3rd edition, 1949, pages 295 and 290, respectively; and conventional pyrophosphate copper baths, as described in U. S. Patents 2,250,556, 2,437,865, and 2,493,092.

The invention may be illustrated by the examples which follow, showing several plating baths, some within and some outside of the invention, their operation, and crack properties of the plate produced by the baths.

## EXAMPLES 1 TO 8

A number of baths, the compositions of which are listed in Table 3, were made up from chromic and sulfuric acids to provide the  $\text{CrO}_3/\text{SO}_4$  ratios noted. Standard steel fatigue test specimens were plated in the baths at the temperature and current density conditions set forth. The specimens were the same, comprising one-half inch round bar stock of SAE 4140 steel. Each specimen was  $3\frac{1}{16}$ " long and had a central portion that was reduced to a diameter of  $1/4$ ". The specimens had been heat-treated and had a hardness of Rockwell C43. The fatigue strength of the specimen steel was 109,000 p. s. i. and the tensile strength was 222,500 p. s. i. Crack-lines were determined by microscopically examining the surface of a specimen at 600X: an arbitrary straight line one inch long was selected in the microscopic field and the average number of crack-lines, including filled-in lines, which crossed such arbitrary line was counted.

Table 3

| Exam.<br>No. | $\text{CrO}_3$ ,<br>g./l. | Ratio:<br>$\text{CrO}_3$ to<br>$\text{SO}_4$ | Temp.,<br>°F. | C. D.,<br>a. s. i. | Thickness,<br>mils | Crack-<br>lines per<br>in. |       |
|--------------|---------------------------|----------------------------------------------|---------------|--------------------|--------------------|----------------------------|-------|
| 35           |                           |                                              |               |                    |                    |                            |       |
| 1            | 250                       | 100                                          | 130           | 2                  | 2                  | 400                        |       |
| 2            | 250                       | 85                                           | 130           | 2                  | 6 to 7             | 1,200                      |       |
| 3            | 250                       | 70                                           | 130           | 2                  | 6 to 7             | 1,200                      |       |
| 4            | 250                       | 55                                           | 130           | 2                  | 6 to 7             | 1,400                      |       |
| 5            | 250                       | 40                                           | 130           | 2                  | 6 to 7             | 1,600                      |       |
| 6            | 250                       | 100                                          | 150           | 2.9                | 2                  | 50                         |       |
| 1            | 250                       | 100                                          | 130           | 2                  | 2                  | 400                        |       |
| 40           | 7                         | 250                                          | 100           | 110                | 2                  | 2                          | 1,200 |
| 5            | 250                       | 40                                           | 130           | 2                  | 6 to 7             | 1,600                      |       |
| 8            | 250                       | 40                                           | 120           | 2                  | 6 to 7             | >1,600                     |       |

As shown by Examples 1 to 5, as the  $\text{CrO}_3$  to sulphate ratio is decreased, the number of crack-lines per inch increases, the temperature being constant. If the ratio is held constant, and the temperature is decreased, the number of crack-lines increases, as shown by Examples 6, 1 and 7, and also by Examples 5 and 8. In these last two groups of examples, the listing of Examples 1 and 5 are repeated merely to illustrate the relationship more readily. Example 1 represents a standard or conventional sulphate bath operated at standard conditions, and as is apparent, it does not produce a plate having the desired number of crack-lines. Example 6, like Example 1, also illustrates a plate not within the invention, the temperature in both examples being too high. Fatigue strengths of specimens plated according to Examples 1 and 8, except that thicker deposits were plated, are compared in Example 9.

## EXAMPLE 9

Test specimens of the kind described were plated according to Examples 1 and 8, except that thicknesses of 10 and 11.6 mils, respectively, were deposited on the specimens. Fatigue strengths of the plated specimens were determined with a rotating beam fatigue machine of the R. R. Moore type. The specimen plated according to Example 1 had a fatigue strength of 57,000 p. s. i., while that plated according to Example 8 had a strength of 67,500 p. s. i.

Unless otherwise specified, the reference in the claims to the  $\text{CrO}_3$  content of the baths is intended to include the amount of  $\text{CrO}_3$  added per se and the amount added in the form of a chromate or dichromate salt.

In the light of the foregoing description, the following is claimed:

1. A method for reducing the loss of fatigue strength following chromium plating of an article of hard steel comprising electrodepositing chromium on the article by passing a current of  $\frac{1}{4}$  to 5 a. s. i. to said article as cathode in an aqueous chromium plating bath at a temperature of 90 to 110° F., said bath having a  $\text{CrO}_3$  content of 100 to 400 g./l. and containing dissolved sulfate,  $\text{SO}_4^{=}$ , as catalyst, the ratio of  $\text{CrO}_3$  to dissolved sulfate being 100:1 to 40:1, plating chromium on the article to form a deposit at least 1 mil thick, said deposit being characterized by having at least 1000 crack-lines per inch and a stress below +5,000 p. s. i., and thereby producing a chromium plated article of hard steel having a fatigue strength of at least 60% of that of the original unplated steel.

2. A method for reducing the loss of fatigue strength following chromium plating of an article of steel having a hardness of at least 20C Rockwell and a fatigue strength of at least 50,000 p. s. i., comprising electrodepositing chromium on the article by passing a current of  $\frac{1}{4}$  to 5 a. s. i. to said article as cathode in an aqueous chromium plating bath at a temperature of 90 to 110° F., said bath having a  $\text{CrO}_3$  content of 100 to 400 g./l. and containing dissolved sulfate,  $\text{SO}_4^{=}$ , as catalyst, the ratio of  $\text{CrO}_3$  to dissolved sulfate being 100:1 to 40:1, plating chromium on the article to form a deposit about 1 to 30 mils thick, said deposit being characterized by having 1000 to 10,000 crack-lines per inch and a stress of +5,000 to -20,000 p. s. i., and thereby producing a chromium plated article of hard steel having a fatigue strength of at least 60% of that of the original unplated steel.

3. A method for reducing the loss of fatigue strength following chromium plating of an article of steel having a hardness of 33C to 47C Rockwell and a fatigue strength of 70,000 to 110,000 p. s. i., comprising electrodepositing chromium on the article by passing a current of  $\frac{1}{4}$  to 3 a. s. i. to said article as cathode in an aqueous chromium plating bath at a temperature of 90 to 130° F., said bath having a  $\text{CrO}_3$  content of 150 to 300 g./l. and containing dissolved sulfate,  $\text{SO}_4^{=}$ , as catalyst, the ratio of  $\text{CrO}_3$  to dissolved sulfate being 85:1 to 40:1, plating chromium on the article to form a deposit about 2 to 15 mils thick, said deposit being characterized by having 1200 to 10,000 crack-lines per inch and a stress of 0 to -20,000 p. s. i., and thereby producing a chromium plated article of hard steel having a fatigue strength of at least 70% of that of the original unplated steel.

4. A method for reducing the loss of fatigue strength following chromium plating of an article of hard steel comprising electrodepositing chromium on the article by passing a current of  $\frac{1}{4}$  to 5 a. s. i. to said article as cathode in an aqueous chromium plating bath at a temperature of 90 to 110° F., said bath having a  $\text{CrO}_3$  content of 300 to 400 g./l. and containing dissolved sulfate,  $\text{SO}_4^{=}$ , as catalyst, said bath containing calcium sul-

fate as the source of said dissolved sulfate, the amount of calcium sulfate being sufficient to saturate the bath and to provide an undissolved excess of calcium sulfate, said bath also containing a soluble calcium compound in an amount sufficient to suppress the concentration of dissolved sulfate from the unsuppressed saturation concentration of the latter to a lower value corresponding to a ratio of  $\text{CrO}_3$  to dissolved sulfate of 100:1 to 40:1, plating chromium on the article to form a deposit at least 1 mil thick, said deposit being characterized by having at least 1000 crack-lines per inch and a stress below +5,000 p. s. i., and thereby producing a chromium plated article of hard steel having a fatigue strength of at least 60% of that of the original unplated steel.

5. The method of claim 1 wherein, prior to chromium plating, a copper strike is deposited on said steel article to minimize any embrittlement of the steel article in said chromium plating bath.

6. The method of claim 1 wherein the steel of said unplated article has a hardness of at least 33C Rockwell.

7. The method of claim 1 wherein the fatigue strength of the steel of said unplated article is 60,000 to 110,000 p. s. i.

8. The method of claim 1 wherein said chromium deposit is at least 5 mils thick.

9. The method of claim 1 wherein said chromium plated article of hard steel has a fatigue strength of at least 70% of that of the original unplated steel.

10. The method of claim 1 wherein said sulfate,  $\text{SO}_4^{=}$ , comprises substantially the entire catalyst in said bath.

11. A method for reducing the loss of fatigue strength following chromium plating of an article of hard steel comprising electrodepositing chromium on the article by passing a current of  $\frac{1}{4}$  to 5 a. s. i. to said article as

cathode in an aqueous chromium plating bath at a temperature of 90 to 130° F., said bath having a  $\text{CrO}_3$  content of 300 to 400 g./l. and containing dissolved sulfate,  $\text{SO}_4^{=}$ , as catalyst, said bath containing calcium sulfate as the source of said dissolved sulfate, the amount

of calcium sulfate being sufficient to saturate the bath and to provide an undissolved excess of calcium sulfate, said bath also containing a soluble calcium compound in an amount sufficient to suppress the concentration of dissolved sulfate from the unsuppressed saturation con-

centration of the latter to a lower value corresponding to a ratio of  $\text{CrO}_3$  to dissolved sulfate of 85:1 to 40:1, plating chromium on the article to form a deposit at least 1 mil thick, said deposit being characterized by having at least 1000 crack-lines per inch and a stress

below +5,000 p. s. i., and thereby producing a chromium plated article of hard steel having a fatigue strength of at least 60% of that of the original unplated steel.

References Cited in the file of this patent

UNITED STATES PATENTS

- |           |                |       |               |
|-----------|----------------|-------|---------------|
| 2,640,021 | Passal         | ----- | May 26, 1953  |
| 2,640,022 | Stareck        | ----- | May 26, 1953  |
| 2,686,756 | Stareck et al. | ----- | Aug. 17, 1954 |